

May 27, 1930.

W. B. BRONANDER

1,760,630

SCRAPER BLADE AND PROCESS OF HARDENING THE SAME

Filed May 17, 1928



INVENTOR

Wilhelm B. Bronander  
BY  
Sydney J. Prescott

ATTORNEY

## UNITED STATES PATENT OFFICE

WILHELM B. BRONANDER, OF MONTCLAIR, NEW JERSEY, ASSIGNEE TO STANDARD TOBACCO STEMMER COMPANY, A CORPORATION OF VIRGINIA

## SCRAPER BLADE AND PROCESS OF HARDENING THE SAME

Application filed May 17, 1928. Serial No. 278,386.

This invention relates to scraper blades and a process of hardening the same, and is particularly applicable to the blades used as inserts on the beater drums of tobacco stemmers and similar machines.

Heretofore, in machines of this type, it has been found difficult to provide insert blades having edges sufficiently hard and permanent to resist undue wear caused by the grit in the tobacco leaves. Blades made entirely of hardened steel have been unsatisfactory because they are brittle and cannot be straightened. Also blades having the working edge only hardened, have likewise proved unsatisfactory because, due to unequal internal strains, the blade warps; moreover, the hardened edge tends to round off at the corners. Another difficulty encountered in making blades for machines of this type has been in making the blades in the same machine uniform. Lack of uniformity causes uneven wear and hence uneven operation of the machine.

Accordingly, the principal object of this invention is the production of scraper blades for tobacco stemmers and other scraping devices, which are uniform, free from the tendency to warp and have permanent self sharpening edges hardened where the wear is greatest. With this and other objects not specifically mentioned in view, the invention consists in certain constructions and combinations which will be hereinafter fully described and then specifically set forth in the appended claims.

In the accompanying drawings:

Fig. 1 is a side elevation of one of the blades used in a beater drum of tobacco stemmers;

Fig. 2 is an end elevation showing a bundle of blades constituting one unit ready for hardening by the improved process;

Fig. 3 is a side elevation of the blade unit after notching of the blades; and

Fig. 4 is an enlarged view showing the completed blades as attached to the drum of the tobacco stemmer.

In carrying the invention into effect, there is provided a blade of substantial thickness along one edge, having a hardened marginal surface on said blade and extending along

said edge, portions of the edge being cut away to form a working edge having hardened corners and a relatively soft central portion. Preferably a series of notches for receiving tobacco stems are cut in said edge so that the parts of the edge engaging the stems have said hardened corners and relatively soft central portions. The process used in producing a set of these blades consists in providing a plurality of blades, covering the surfaces thereof, except the edge portions to be hardened, temporarily securing said blades together in spaced relation to form a single unit and subjecting the unit to a surface hardening operation. In the best mode of carrying out the invention, the edges of said blades subjected to the surface hardening operations are cut away to provide a working edge having hardened corners and a relatively soft central portion. The method and means above referred to may be widely varied in construction within the scope of the claims, for the particular method and means selected to illustrate the invention is but one of many possible embodiments of the same. The invention, therefore, is not to be restricted to the precise details of the structure shown and described.

Referring to the drawings, a number of blades 5 of substantial thickness at their edge portions 6, which in the present embodiment are of high carbon steel, such as tool steel, are assembled in a unit having the spacers 10 between the successive blades, the blades and spaces being held together between the cover plates 11 by the bolts 12 passing through the holes 9 of the plates. The number of blades in the stack is equal to the number required for a complete set of blades for the stemming machine, so that every blade of the set will get exactly the same treatment, with the result that any wear will uniformly affect all of the blades. The spacers 10 and the cover plates 11 are made of such width as to cover all the side surfaces of the blade, except two opposite longitudinal marginal portions of equal width and the edge portions thereof, the surfaces of which are to be hardened.

In the method selected to illustrate the invention, this unit is immersed in a bath of po-

55

60

65

70

75

80

85

90

95

100

tassium cyanide, in which it is heated to a temperature of around 1500 degrees Fahrenheit, more or less, for 15 or 20 minutes. It is then exposed to air of ordinary room temperature for a very short time, 20 or 30 seconds, to normalize the steel, after which it is quenched in oil. This will result in a thin hardened surface portion or skin on the exposed parts of the blade. Other methods of hardening the surface portions of the blade 10 may be used. For instance, blades of low carbon, or machine steel, may be utilized and the parts which it is desired to harden, may be surface carbonized, whereby subsequent hardening will result in hardening the carbonized surface only. The exposed edge portions of the blades, after being subjected to the hardening operation, or to an essential part thereof, have notches 7 cut therein, as shown in Figs. 3 and 4.

20 For this purpose, the blades may be disassembled from the unit and the notches cut out in any suitable way, or the blades may be notched while in the unit, as shown in Fig. 3. 25 The notches of each successive blade are offset to give a spiral arrangement of notches, when the blades are assembled on the drums of the stemmer machine.

As will be seen from Fig. 4, showing the 30 blades as mounted on the holder 8 of the drum of the stemmer machine, the notches 7 cut in the edge of the blade 5 will cut away the hardened surface portion of the edge 6 to form a stem engaging edge parts having hardened 35 corners 13 formed by the hardened surfaces 13, and a relatively soft central portion 7.

As shown in Fig. 4, the scraping operation 40 of the blade on the stem of the tobacco leaf will result in this softer central portion of the notched edge being washed away or hollowed out, leaving the thin edges of the hardened 45 surface portions 13 exposed, thus rendering the blades self sharpening by maintaining hard sharp corners on the stem engaging edges of the blades.

It is noted that by hardening equal widths 50 at the margins of the blades, the strains caused by shrinking of the blades in cooling will be neutralized. The soft center also serves to neutralize such strains and because only thin 55 surface portions of the blades are hardened, the blades can be straightened without danger of breaking them.

What is claimed is:

55 1. A self sharpening scraper element, comprising a blade of substantial thickness along one edge having hardened marginal surfaces on each side of said blade and extending along said edge, portions of the edge being cut away 60 to form a working edge having hardened corners and a relatively soft central portion.

2. A self sharpening scraper element, comprising a blade of substantial thickness along one edge having hardened marginal surfaces 65 on each side of said blade and extending along

said edge, portions of the edge being cut away to form a working edge having hardened corners and a relatively soft central portion, said blade being provided with similar marginal surfaces similarly located along the opposite 70 edge of said blade to prevent warping.

3. An insert for tobacco stemmers comprising a case hardened blade having an edge portion of substantial thickness, and a series of notches for receiving the tobacco stems cut 75 in said edge portion so that the parts of the edge engaging the stems have hardened corners and relatively soft central portions.

4. An insert for tobacco stemmers comprising a blade of substantial thickness along one 80 edge and having hardened marginal surfaces one on each side of the blade and extending along said edge, said blades being provided with similar marginal portions similarly located along the opposite edge of the blade to prevent warping, the former edge having 85 notches cut therein to receive the stem, so that the parts of the edge engaging the stems have hardened corners and relatively soft central portions.

90 In testimony whereof, I have signed my name to this specification.

WILHELM B. BRONANDER.

70

75

80

85

90

95

100

105

110

115

120

125

130